

## 1

3,454,420

**WATERPROOFED ORGANIC FIBROUS PRODUCTS**  
Jacques Pierre Edmond Pechmeze, Paris, and Gérard Léon Alphonse Mangeney, Deuil-la-Barre, France, as signors to Etablissements Kuhlmann, Paris, France  
No Drawing. Filed Jan. 5, 1966, Ser. No. 518,800  
Claims priority, application France, Jan. 12, 1965,

1,570

Int. Cl. B44d 1/00

U.S. Cl. 117—121

7 Claims

### ABSTRACT OF THE DISCLOSURE

Organic fibrous materials which have been waterproofed by the reaction product of an acid halide having a hydrocarbon chain of 14 to 22 carbon atoms and a metal alcoholate.

The present invention is concerned with new waterproofing products which are soluble in those organic solvents used in drycleaning. Such products are very useful when the cleaned articles have to be made waterproof or kept waterproof.

However, the waterproofing effect has been achieved it is not resistant to, or at least has very poor resistance to, drycleaning hence the necessity to subject the cleaned article to a subsequent reproofing. This treatment may be effected by means of the ordinary commercial waterproofing substances, such as those based on emulsions of paraffin wax, stearoylaminomethyl-pyridinium chloride, stearylhydroxymethyl-pyridinium chloride or chromium stearato-chloride. These products must be applied from an aqueous bath. Now the reason for cleaning with solvents is in fact to avoid all manipulation of the clothes in an aqueous medium, which may be harmful to their appearance and cause felting or shrinking, making them finally unusable. It is therefore of importance to make available to dyers and cleaners waterproofing substances which are soluble in the solvents which they use such as, for example trichloroethylene, perchlorethylene, white spirit, or dry cleaning solvent.

Such products have already been proposed. There may be mentioned, for example, organic derivatives of the metals of Groups III or IV, which may be in the form of salts of aliphatic acids of high molecular weight, in the form of alcoholates of lower aliphatic alcohols, or in the form of products resulting from the action of aliphatic acids of high molecular weight on these alcoholates. Waterproofing products obtained from alcoholates of polyvalent metals and phosphoric esters, in particular, have been described, and intended more especially for the waterproofing of leather.

Among all these products, some have a very low solubility in the drycleaning solvents and for this reason are difficult to use. Others, on the contrary, are too soluble in these same solvents with the result that during the drying of the treated articles, there is a migration of the product on the textile surface, which causes rings and spots.

We have found that waterproofing products having an excellent solubility in all the solvents used for drycleaning and giving an excellent waterproofing effect without

## 2

alteration of the appearance of the treated articles, can be obtained by reacting an acid halide which contains a hydrocarbon chain with 14 to 22 inclusive carbon atoms with an alcoholate of a metal of Group III or IV of the Periodic Classification at high temperature.

Examples of acid halide which may be used to carry out the invention are the chlorides of aliphatic carboxylic acids in which the hydrocarbon chain contains 14 to 22 carbon atoms, such as the higher fatty acids of natural origin, the acids resulting from the oxidation of paraffins or oxo aldehydes, or Koch acids, or the chlorides of alkylsulphonic acids resulting from the sulphochlorination of paraffins and containing 14 to 22 carbon atoms, or the chlorides of phosphoric acid in which one or two acid groups have been esterified by aliphatic alcohols with a hydrocarbon chain containing 14 to 22 carbon atoms, such as the fatty alcohols of natural origin or the oxo alcohols, or the chlorocarbonates of these same alcohols.

Examples of the metal alcoholates which may be used are the alcoholates of aluminum, zirconium or titanium, in which the alcoholic radicals are those of ethyl, isopropyl, propyl, normal butyl, isobutyl, 2-ethylhexyl, lauryl or oxo alcohols.

The following procedure may be used for example in the preparation of the products of the invention. A solution of a metal alcoholate in an inert solvent, such as for example toluene, is slowly added at low temperature, for example below 50° C., to a solution in the same inert solvent of the acid halide. The amount of metal alcoholate added is such that it corresponds to one molecular equivalent per atomic equivalent of halogen present in the acid halide. When the addition is completed, the solvent is driven off by distillation. The mass remaining is then heated with agitation at a temperature between 140° C. and 160° C., preferably between 150° C. and 160° C. The separation of alkyl halide, the hydrocarbon chain of which corresponds to that of the alcohol of the metal alcoholate, the ether corresponding to the same alcohol, as well as the alcohol resulting from the alcoholate is then noted. The heating is interrupted when this distillation ceases. The product remaining in the apparatus constitutes the waterproofing product of the invention.

The waterproofing products thus obtained are soluble in trichlorethylene, perchlorethylene, white spirit, and drycleaning solvent. Their solutions in these solvents enable textile materials to be made waterproof or their waterproof properties to be preserved if they already possess them. These solutions may also be used for the waterproofing of other fibrous materials such as leather.

In the following examples which are purely illustrative the parts given are parts by weight, unless the contrary is indicated.

### EXAMPLE 1

151.25 parts of stearoyl chloride and 125 parts by volume of toluene are introduced into an apparatus fitted with a mechanical stirrer, a thermometer, a gauge, and a plunging tube. 102 parts of aluminum isopropylate in solution in 125 parts by volume of toluene are added by means of the gauge in a period of 4 hours. During this addition the temperature of the mass rises from 24° C. to 40° C. When the introduction is completed, the toluene is distilled

off under reduced pressure, the temperature of the mass being maintained at 40° C.

After the distillation, a Dean-Stark separating tube is fitted on the apparatus. The exit of the condenser is connected to tubes or flasks plunged into carbon dioxide snow. A stream of nitrogen is passed into the mass by means of the plunging tube and the mass is heated to 145–150° C. A colourless liquid distils over and is collected in the Dean-Stark tube and in the tubes or flasks plunged in the carbon dioxide snow. 47 parts of a liquid containing isopropyl chloride, isopropyl ether and isopropanol are obtained. Then the distillation ceases, the heating is interrupted, and the mass is allowed to cool under a stream of nitrogen. The residue consists of 206 parts of a very thick brown liquid containing 6.46% of Cl and 6.30% of Al. The product thus obtained is excellently soluble in chlorinated solvents and aliphatic hydrocarbons, and its solutions give waterproof properties to fabrics.

#### EXAMPLE 2

The operation is as in Example 1, but the 102 parts of aluminium isopropylate are replaced by 170 parts of titanium tetrabutylate. 275 parts of a very thick brown product of resinous consistency, containing 4.72% of Cl and 8.70% of Ti, are obtained. It is excellently soluble in all the solvents customarily used for drycleaning. Its solutions give excellent waterproof properties to clothes.

#### EXAMPLE 3

399 parts of stearyl dichlorophosphate (dichlorophosphate of technical stearyl alcohol) and 500 parts by volume of toluene are introduced into an apparatus fitted with a mechanical stirrer, a thermometer, a gauge, a plunging tube and a reflux condenser. 408 parts of aluminium isopropylate in solution in 700 parts by volume of toluene are added by means of the gauge in a period of 4 hours. The temperature of the mass rises from 20° C. to 55° C. After this introduction, the toluene is driven off by distilling under reduced pressure, the mass being heated to 40° C.

When all the toluene has been eliminated, a Dean-Stark separating tube is fitted on the apparatus and the outlet of the condenser is connected to bubblers plunged into the carbon dioxide snow. A stream of nitrogen is passed into the mass by means of the plunging tube and the temperature is raised to 155° C. When the temperature reaches 130° C., a colourless liquid begins to distil and is collected in the Dean-Stark tube and in the bubblers. Heating is continued until all distillation ceases. 107 parts of this colourless liquid are thus obtained, which on analysis is found to be composed of isopropyl chloride, isopropyl ether and isopropanol.

After cooling, there remain in the flask 700 parts of a very thick, dark brown liquid, containing 6.47% of Cl, 4.15% of P and 7.7% of Al, which is excellently soluble in chlorinated solvents and in aliphatic hydrocarbons.

#### EXAMPLE 4

620.5 parts of octadecyl chlorophosphate and 700 parts by volume of toluene are introduced into an apparatus identical with that of Example 3. 204 parts of aluminium isopropylate in solution in 350 parts by volume of toluene are added by means of the gauge in a period of 4 hours. The operation is carried out in the same way as that of Example 3. 770 parts of a brown, very thick, resinous product are obtained, which is excellently soluble in the solvents used for drycleaning and contains 2.30% of Cl, 4.02% of P and 3.50% of Al.

#### EXAMPLE 5

399 parts of stearyl dichlorophosphate and 500 parts by volume of toluene are introduced into an apparatus fitted with a mechanical stirrer, a thermometer, a plunging tube, and a gauge. A solution of 542 parts of zirconium tetraethylate in 700 parts by volume of toluene

is introduced by means of the gauge in a period of 4 hours. The operation is finished by the method described in Example 3. 830 parts of a dark, resinous, very thick product, soluble in the solvents used for drycleaning and containing 3.73% of P, 4.2% of Cl and 10.80% of Zr, are obtained.

#### EXAMPLE 6

A piece of cotton satin weighing 300 g./m.<sup>2</sup> is treated in a bath of perchlorethylene containing 30 g. per litre of the waterproofing product of Example 1. After drying and returning to the usual atmospheric humidity, the fabric possesses excellent waterproof properties characterised by a Schmerber figure equal to 350 and a spray test equal to 100.

#### EXAMPLE 7

A piece of cotton satin weighting 300 g./m.<sup>2</sup> is impregnated in a bath of perchlorethylene containing 20 g. per litre of the waterproofing product described in Example 3 and 20 g. per litre of paraffin wax having a melting point between 54° C. and 58° C. After draining, drying and returning to the usual atmospheric humidity, the fabric possesses remarkable waterproof properties, characterised by a Schmerber figure equal to 374 and a spray test equal to 100. In addition, the initial appearance of the fabric has not been modified in any way.

#### EXAMPLE 8

A piece of cotton satin weighing 300 g./m.<sup>2</sup> is treated in a bath of white spirit containing 10 g. per litre of the waterproofing product described in Example 4 and 30 g. per litre of paraffin wax having a melting point between 54° C. and 58° C. After draining, drying and taking up the usual atmospheric humidity, the fabric possesses waterproof properties characterised by a Schmerber figure equal to 365 and a spray test equal to 100.

#### EXAMPLE 9

A piece of calico weighing about 100 g./m.<sup>2</sup> is impregnated in a bath of perchlorethylene containing 30 g. per litre of the waterproofing product described in Example 3. After drying and taking up the usual atmospheric humidity, the calico is excellently waterproof. It possesses a Schmerber figure equal to 203 and a spray test equal to 100.

We claim:

1. Organic fibrous materials waterproofed by means of a product resulting from the reaction at high temperature between an acid halide having a hydrocarbon chain having from 14 to 22 carbon atoms and a metal alcoholate, the metal of which is selected from the group consisting of aluminium, zirconium, and titanium, the amount of the said metal alcoholate being in a ratio of 1 molecular equivalent per atomic equivalent of halogen present in the acid halide.
2. The waterproofed fibrous material as defined in claim 1 wherein the alcoholic radical of the metal alcoholate is derived from ethyl, propyl, isopropyl, normal butyl, isobutyl, 2-ethylhexyl, lauryl, or an oxo alcohol.
3. The waterproofed fibrous material as defined in claim 1 wherein the acid halide is stearoyl chloride and the metal alcoholate is aluminium isopropylate.
4. The waterproofed fibrous material as defined in claim 1 wherein the acid halide is stearyl dichlorophosphate and the metal alcoholate is aluminium isopropylate.
5. The waterproofed fibrous material as defined in claim 1 wherein the reaction between the acid halide and the metal alcoholate is effected at a temperature between 140° C. and 160° C.
6. The waterproofed fibrous material as defined in claim 5 wherein the temperature is between 150° C. and 160° C.
7. The waterproofed fibrous material as defined in claim 1 wherein said acid halide is a member selected from the group consisting of

- (a) a chloride of an aliphatic carboxylic acid in which the hydrocarbon chain has from 14 to 22 carbon atoms,
- (b) a chloride of phosphoric acid in which one or two acid groups have been esterified by an aliphatic alcohol having a hydrocarbon chain of from 14 to 22 carbon atoms,
- (c) a chloride of an alkylphonic acid having 14 to 22 carbon atoms, and
- (d) a chlorocarbonate of an aliphatic alcohol having 10 a carbon chain of from 14 to 22 carbon atoms.

## References Cited

## UNITED STATES PATENTS

|           |         |                      |           |
|-----------|---------|----------------------|-----------|
| 2,774,689 | 12/1956 | Orthner et al. ----- | 117—135.5 |
| 2,838,422 | 6/1958  | Orthner et al. ----- | 117—135.5 |

WILLIAM D. MARTIN, *Primary Examiner.*

THEODORE G. DAVIS, *Assistant Examiner.*

U.S. Cl. X.R.

117—135.5, 142, 143